# EUROPEAN PATENT APPLICATION

(11) **EP 0 521 638 A1**
(43) Date of publication of application: **07.01.1993**
(21) Application number: 92305608.9
(22) Date of filing: 18.06.1992
(51) Int. Cl.: C10M 171/00

(54) **Electrorheological fluid comprising a polysiloxane having a fluorohexylalkyl group**

(30) Priority: 29.06.1991 GB 9114102
(71) Applicant: Dow Corning Limited, South Glamorgan CF6 7YL Wales (GB)
(72) Inventor: Rowlands, Martin, Neath, West Glamorgan SA11 3UD (GB)
(74) Representative: Bullows, Michael

(57) **Abstract**

An electrorheological fluid which is a suspension of a finely divided solid in an insulating fluid comprising fluorohexylalkyl functional polysiloxane.

## Description

This invention is directed to an electrorheological fluid which is a suspension of a finely divided solid in an insulating fluid. More particularly, the invention is related to the use of a polysiloxane having a fluorohexylalkyl group as the insulating fluid.

Electrorheological fluids are well known in the art and are suspensions of finely divided polyelectrolyte solids in an insulating fluid. Electrorheological fluids possess the remarkable property in that when the fluid is subjected to a strong electrical field, their rheological properties change from that of a free flowing liquid to a Bingham type material. Thus, upon application of a strong electrical field, the fluid undergoes a significant viscosity increase that is reversible upon removal of the field.

It has been proposed to employ certain fluorosilicones as insulating fluids in electrorheological applications. For example, U.S. Patent 4,812,251 (Stangroom) dated 14th March 1989 discloses an electrorheological fluid comprising a hydrophilic solid and a hydrophobic liquid component in which the liquid component comprises a fluorosilicone having an average molecular weight of 200 to 700. The low molecular weight fluorosilicones disclosed are exemplified by a mixture of linear and cyclic polysiloxanes, primarily methyl trifluoropropyl siloxanes, the linear chains having trimethylsilyl end groups. U.S. 4,812,251 teaches that these fluorosilicones are of low viscosity and are miscible with polychlorotrifluoroethylene to provide low viscosity mixtures having appropriate density matching with solids e.g. starch or silica gel used to prepare electrorheological fluids.

G.B. 2 210 893 A (American Cyanamid) dated 21st June 1989 discloses an electrorheological fluid comprising a solid phase (for example the lithium salt of a polymethacrylic acid) dispersed in a base liquid comprising a polyfluoroalkylmethylsiloxane. These polysiloxanes are exemplified by (CH₃)₃Si(CH₃RSiO)ₙSi(CH₃)₃ where R represents 3,3,3-trifluoropropylsiloxane (i.e. R represents -CH₂CH₂CF₃) and n has a value such that the material is a liquid having an average molecular weight from 500 to 1500. Polymethyl 1,1,2,2-tetrahydroperfluorooctylsiloxane is also referred to, but no specific examples of such materials are exemplified. The base liquid may have a viscosity up to about 10,000 cSt at 25°C; low viscosities are mentioned and viscosities of greater than 100 cSt are exemplified.

It is understood that in some respects the known polymethyl 3,3,3-trifluoropropylsiloxane base liquids are more efficient than many other fluids, for example in respect of static yield stress. However, even these materials have a comparatively high current demand i.e. the current density required to activate the fluid at a particular field. The lower the current demand, the less power is required to convert the fluid to a Bingham type material. An insulating fluid exhibiting a low current demand would be highly advantageous in a commercial electrorheological device.

It has now been found that an improved insulating fluid for use in an electrorheological application can be provided by use of certain high density, low viscosity, polysiloxanes having at least one silicon-bonded fluorohexylalkyl group.

The present invention provides in one of its aspects an electrorheological fluid comprising a suspension of a finely divided solid in an insulating fluid comprising a polysiloxane having at least one siloxane unit having a silicon-bonded fluorohexylalkyl group.

An electrorheological fluid according to the present invention comprises an insulating fluid comprising a polysiloxane having at least one siloxane unit having a silicon-bonded fluorohexylalkyl group i.e. a fluorohexylalkyl functional polysiloxane. The polysiloxane preferably has a high density to match the density of the finely divided solid, i.e. a density greater than about 1.3g/ml and a low viscosity, i.e. lower than about 100 cSt, more preferably lower than about 40 cSt at 25°C. Preferred polysiloxanes have a density of at least 1.40 g/ml and a viscosity not in excess of about thirty centistokes measured at 25°C.

Preferred polysiloxanes have the general formula R₃SiO[(R₂SiO)ₓ(RR'SiO)_{y}]ₙSiR₃ in which R is an alkyl radical having from one to six carbon atoms, R' represents the group -CH₂CH₂(CF₂)₄F, x has a value of 0 to 0.5; y has a value of 1 - x and n has a value of 3 to 10. Preferably the alkyl groups are all methyl groups.

Polymethylsiloxanes for use in the present invention may be prepared from a fluorohexylmethyl silicone hydrolyzate (II) produced by hydrolysis of a mixture of dimethyldichlorosilane and fluorohexylmethyldichlorosilane according to the scheme
Equilibration of the fluorohexylmethyl/silicone hydrolyzate (II) with hexamethyldisiloxane and trifluoromethasulphonic acid as a catalyst, produces a stable trimethyl end-blocked, fluorinated siloxane thus:
One of the preferred fluoro-hexylalkyl functional polysiloxanes is the compound of the formula Me₃SiO[(Me₂SiO)_{0.2}(MeR'SiO)_{0.8}]₇SiMe₃ in which Me represents the methyl group.

While it is possible to employ various materials for example silica gel, starch, poly-methacrylic acid and phenolformaldehyde solids as the finely divided solid in the insulating fluid, the finely divided solid most preferred in accordance with the present invention is poly(acenequinone)
hereinafter referrred to as PAQR. PAQR is a black polymeric solid and a range of thermally and environmentally stable poly(acenequinones) is commercially available, with conductivities varying from 10⁻⁴ to 10⁻¹¹ Scm⁻¹. The preferred PAQR powder has a density of about 1.4g/ml. The PAQR should have a particle size of between one and fifty microns in order to facilitate the dispersibility of the particles in the insulating fluid, preferably less than about twenty microns in diameter. The finely divided PAQR may be present in the electrorheological fluid in an amount of from 20 to 60 percent, preferably about thirty percent on a volume/volume proportion.

Electrorheological fluids according to the invention demonstrate current densities at 3 kV many times lower than the current densities of the order of 300 and 250 µAcm⁻² at 3kV, demonstrated by fluids comprising chlorinated paraffin and PAQR or 3,3,3-trifluoropropylsiloxane and PAQR.

Following is an example illustrating a method of making fluorohexylalkyl functional polysiloxanes suitable for use in the present invention.

### Example I

Into a reaction flask there was mixed 538.1 grams of the fluorohexylmethyl silicone hydrolyzate (II) shown above in Equations (1) and (2) and 61.9 grams of hexamethyldisiloxane. A nitrogen blanket was applied and the flask was heated to 70°C. To the flask was added 0.35 millilitres of trifluoromethane sulfonic acid and sixty microlitres of water. Heating at 68 to 70°C was maintained for five hours. Three millilitres of dimethylformamide was added and heating was maintained for an additional hour. The flask was cooled to below 30°C and 7.5 grams of sodium hydrogen carbonate was added and the contents of the flask were stirred for ten minutes. The flask contents were filtered through DICALITE and stripped for twenty minutes. The product was a water white fluid having a viscosity of 24 centipoise measured at 155 sec⁻¹ and 25°C. The product was identified as
in which Me is methyl.

The advantage provided by the use of the fluorohexylalkyl functional polysiloxanes of this invention was verified by testing four silicone fluids including a fluid of the present invention. The fluids tested were a polydimethylsiloxane identified below as Compound "C", a fluorohexyl functional polysiloxane identified below as Compound "B", a trifluoropropyl functional polysiloxane identified below as Compound "A", and a cyanofunctional polysiloxane identified below as Compound "D". Each of the fluids tested contained a dispersion of a polymeric semiconducting solid and were measured for (i) static yield stress which is a measurement of the rheoelectrical capability of a liquid/solid dispersion, and (ii) current demand which is the power required to produce a rheoelectrical effect. It was found that the perfluorohexyl functional siloxane system of the present invention required significantly less power to produce a rheoelectrical effect than any of the other comparative systems.

The fluids tested are shown below:
(a) Compound A
   - Structure ::
   - Viscosity :: 30mm²/sec
   - Density :: 1.20g/ml
(b) Compound B
   - Structure ::
   - Viscosity :: 30mm²/sec
   - Density :: 1.40g/ml
(c) Compound C
   - Structure :: Polydimethylsiloxane
   - Viscosity :: 350mm²/sec
   - Density :: 1.0g/ml
(d) Compound D
   - Structure ::
   - Viscosity :: 3500mm²/sec
   - Density :: 1.0g.ml
Static yield stresses and current demand were measured on an apparatus in which a fluid sample (2ml) was placed in the bottom section of a split copper cell. The top section of the cell was brought into contact with the fluid and a d.c. field was applied across the cell (distance across fluid = 1mm). The top section was connected to a micrometer and strain gauge and a force was applied using the micrometer, until the top section moved. This force was the static yield stress and was recorded at different applied fields. The current passed was measured using an ammeter and converted to current density, µAcm⁻².

For the purpose of these measurements, the PAQR was dispersed in a 30% v/v proportion, into each sample. Static yield stress and current demand are directly proportional to the percent volume of dispersed polymer and the applied field.

Static yield stress (o) is the shear stress required to induce flow in a material. An electrorheological fluid, when subjected to high field, is transformed from a fluid to a Bingham type material with shear stress under both zero and finite shear rates. Static yield stress, therefore, is a measure of the extent to which a liquid/solid system exhibits an electrorheological effect.

Of the four fluids tested only the cyanofunctional fluid "D"/PAQR failed to show any measurable static yield stress (±200 Pa) up to a field of 2.4 kVmm⁻¹.

Compound "C"/PAQR showed the least effect of the remaining three fluids with a static yield stress of only 1.1kPa at 3.2kVmm⁻¹. The increase in static yield stress with field for "C" was less rapid than with the fluorinated siloxanes "A" and "B". "B"/PAQR AND "A"/PAQR had similar static yield stress/field curves each with a value of over 2 kPa at 3.2 kVmm⁻¹. The fluorinated siloxanes "A" and "B" therefore, are twice as efficient as "C". The static yield stresses mirror the dielectric constants of the fluids and approximate values are given below.

| Fluid | Dielectric Constant |
|---|---|
| PDMS | 3 |
| Fluorinated siloxanes | 6 - 7 |

Chlorinated paraffin/PAQR has a current density of over 300 µAcm⁻², at 3kV, "C"/PAQR was better at 240 µAcm⁻² and similar to the trifluoropropyl functional siloxane system "A"/PAQR with a density of 260 µAcm⁻². At these high levels of insulation, these difference were negligible. The fluorohexyl functional fluid system "B"/PAQR, however, had a current density at 3kV, seventeen times lower than the other fluid systems, 17 times lower than "A"/PAQR and "C"/PAQR and more than 20 times lower than chlorinated paraffin/PAQR.

Currently accepted theories on current demand do not explain lower current density. Two possible reasons for current demand in dry fluids are believed to be that electron-hole migration involving light charge carriers tunnels between the fluids' particles. This should occur to a lesser extent using a fluorohexyl functional siloxane due to its high density (closer packing of particles). The second possible explanation is believed to be that a fluid under field is more ordered than in the absence of a field and hence entropy is lowered. Maintaining order against thermal disordering requires work to be performed and hence power to be drawn. Use of a fluorohexyl functional siloxane base fluid results in either the system being less ordered under field (a situation reflected in a low static yield stress), or less work is required to maintain ordering.

The improved static yield stress and low current demand of "B"/PAQR fluid systems, combined with its high density indicates that fluorohexyl functional siloxanes are superior as base fluids in electrorheology.

## Claims

1. An electrorheological fluid comprising a suspension of a finely divided solid in an insulating fluid comprising a polysiloxane having at least one siloxane unit having a silicon-bonded fluorohexylalkyl group.

2. A fluid according to Claim 1 in which the polysiloxane has a density of at least 1.40 g/ml.

3. A fluid according either one of Claims 1 and 2 in which the polysiloxane has a viscosity not in excess of about thirty centistokes measured at 25°C.

4. A fluid according to any one of the preceding Claims in which the polysiloxane is of the general formula in which R is an alkyl group having one to six carbon atoms; x has a value of 0 to 0.5; y has a value of 1 - x and n has a value of 3 to 10.

5. A fluid according to any one of the preceding Claims in which the polysiloxane is a polymethylsiloxane.

6. A fluid according to Claim 4 in which the fluorohexylalkyl functional polysiloxane has the formula in which Me is methyl.

7. A fluid according to Claim 1 in which the finely divided solid is poly(acenequinone).

8. A fluid according to Claim 7 in which the finely divided solid poly(acenequinone) has a particle size of less than about twenty microns in diameter.

9. A fluid according to Claim 7 in which the finely divided solid poly(acenequinone) is present in the electrorheological fluid in an amount of about 30% by volume.
